

Patented Jan. 29, 1924.

1,481,942

# UNITED STATES PATENT OFFICE.

FELIX A. VOGEL, OF NEW YORK, N. Y., ASSIGNOR TO THE GENERAL FUEL BRIQUETTE CORPORATION, OF NEW YORK; N. Y., A CORPORATION OF NEW YORK.

## FUEL BRIQUETTE AND THE PROCESS OF MAKING SAME.

No Drawing.

Application filed October 18, 1919. Serial No. 330,382.

To all whom it may concern:

Be it known that I, FELIX A. VOGEL, a citizen of the United States, and a resident of the borough of Manhattan, city, county, and State of New York, have invented certain new and useful Improvements in Fuel Briquettes and the Processes of Making Same, of which the following is a specification.

10 The invention relates to the manufacture of fuel briquettes and has for its object the production of such a briquette which will not disintegrate in the presence of moisture.

The problem of producing a fuel briquette 15 of this character is one of long standing. It has heretofore been proposed to mix fuel fines with a large variety of substances or compounds which may be termed binders by reason of their adhesive character.

20 Among such substances are starch, sugar, molasses, sulphite pitch (waste from paper mills) and similar cellulose compounds. These materials called binders, even after the briquette is dried, remain soluble and the

25 briquettes when they subsequently come in contact with moisture or are exposed to rain begin to disintegrate. Various processes have heretofore been adopted for overcoming the difficulty and to cause the production 30 of a briquette which shall be waterproof in character. Some of these efforts have been to render the binder insoluble but none of the suggestions have led to the production of a merchantable waterproof fuel briquette of

35 the binder type. The manner in which I overcome the difficulties hitherto existing is as follows:

Fuel fines are dried according to the usual practice, preferably in a rotary drier.

40 I then add a carbohydrate binder dissolved in a suitable quantity of water in proper proportion. The solution is preferably introduced to the fuel fines in a horizontal paddle-mixer or some other appropriate appliance.

45 The proportion of binder will naturally vary according to its particular characteristic but may generally be stated as being from 4 to 10 per cent. When sulphite pitch is used, the proportion is about 6 to 8

50 per cent. The solution of binder and water and the fuel fines are thoroughly mixed in the paddle-mixer and when the mixing operation is complete, the mixed flux of coal and binder is introduced into a masticator consisting preferably of heavy rolls

revolving in a suitable pan. A type of masticator particularly suitable for the purposes of this invention is the one illustrated in Canadian Patent No. 184,646 of May 28, 1918, to Van Hall, Basenau and Van Haagen. The action of this masticator upon the mixture causes a close digestion and intercompounding of the coal with the binder and the result is that each particle of coal obtains a thin film or coating of the dissolved binder. The application of the principle of mastication to briquettes compounded with a binder also leads to the use of a minimum amount of the binder substance. When the briquette is completed there would consequently be a minimum amount of moisture and soluble binder in the product, which is of material assistance in the fixing or carbonizing operation. The principal of mastication is employed in the Van Hall patent, to which reference has been made, for the purpose of setting up in the coal particles an autogenous cementing quality so that a binder is not required. By employing the mastication principle in connection with a binder, however, a new result is obtained in that by reason of the thin minute coating of binder on each coal particle the ultimate briquette consists of a connected net-work, as it were, composed of the various thin layers of binder solution where they contact with one another. A briquette formed from material thus treated will in effect be a body composed of a multiplicity of minute pockets all connected together and each pocket closed and containing within itself a minute particle of coal or other fuel substance used as the base of the fuel briquette.

55 After the material leaves the masticator it is pressed into the form of briquettes in any standard press in accordance with well known practice.

The briquette in this shape, when dried, will still contain the water soluble binder and will, consequently, not be waterproof, so that it becomes necessary to convert the binder contents of the briquettes into insoluble material. The first step is to remove the moisture but this is not sufficient. It will also be necessary to remove practically all of the hydrogen and oxygen from the binder, leaving only a granular or fibrous structure of carbon which will retain a high binding quality by reason of the fact

that it is fibrous and of close texture. The process consists in passing the briquettes through a suitable heating appliance comprising a series of zones of increasing temperature. Care should be exercised that the heat treatment in the various zones is uniform for each zone. The first zone is maintained at a heat of approximately 300° F. and the briquettes are allowed to remain in 10 this zone for approximately forty minutes. The next zone is maintained at approximately 400° F. and the briquettes are exposed to this temperature for about five minutes. The next zone is maintained at 15 approximately 600° F. and the briquettes are exposed to this temperature for about fifteen minutes. The first zone removes practically all the moisture contents, while the succeeding higher temperatures remove 20 the water of crystallization and the hydrogen and oxygen contents, leaving the carbon content only.

When the procedure is complete the briquette will be waterproof and weatherproof 25 and will be capable of being handled and transported in a commercial way without disintegration. The briquette, when finished, will consist of a net-work of extremely fine-textured carbon, supporting in its 30 interstices minute particles of coal or other fuel. The structure of the carbon in this briquette is different from the structure of the carbon of prior briquettes in that it is fibrous and fine-textured, whereas the carbon in prior briquettes has been non-fibrous, 35 granular and deficient in tenacious, cohesive faculty. I attribute the result which I obtain to the circumstance that I use a limited volume of binding material,—less than 40 would be required to produce, by itself, a properly cohering briquette upon mere mixing of the fuel and the binder without subsequent intermastication. The result of using so little of the binding material and 45 nevertheless of distributing it completely throughout the fuel compels the formation of a universally distributed, exceedingly thin film of binding substance which coats practically each particle of the fuel without 50 anywhere existing in the mass in the form of an accumulation or a drop of the binder. Upon subsequent carbonization there is produced a carbonized mesh of such small transverse dimension as to be almost unmeasurable, which mesh extends, however, 55 throughout the entire briquette and is of special and unique character, which manifests itself in the ultimate result as a fibrous, fine-textured carbon which tenaciously holds 60 together and assists materially in securing permanence of the briquette as such. After the briquettes have received the last heat treatment, they may be subjected to a cooling treatment in which either water or air 65 may be used as the cooling medium so that

the briquettes will become sufficiently cool to allow of immediate storage.

What I claim is:

1. In the art of producing briquettes that improvement which consists in mixing finely comminuted particles of a substance to be briquetted with a relatively small proportion of a dissolved water soluble binding substance, sufficient in quantity but limited to supply only a coating of the particles upon the subsequent masticating treatment, coating each of the particles to be briquetted with a minute film of the binding solution by subjecting the mixture to a masticating action until no accumulation of the binder 70 as such exists in the mixture but the whole of said binder has been converted into a thin film extending throughout the mass of the material, then forming the material into briquettes, removing the moisture therefrom 75 and carbonizing the binder.

2. In the art of producing fuel briquettes that improvement which consists in mixing finely comminuted fuel with a relatively small proportion of a dissolved water soluble binding substance, sufficient in quantity 80 but limited to supply only a coating of the particles upon the subsequent masticating treatment, coating each particle of the fuel with a minute film of the binding solution 85 by subjecting the mixture to a masticating action until no accumulation of the binder as such exists in the mixture but the whole of said binder has been converted into a thin film extending throughout the mass of the 90 material, then forming the material into briquettes and subjecting the briquettes to successive stages of increasing heat to remove moisture and to carbonize the binder 95

3. In the art of producing fuel briquettes that improvement which consists in mixing finely comminuted fuel with a relatively small proportion of a dissolved water-soluble binding substance, sufficient in quantity 100 but limited to supply only a coating of the fuel particles upon the subsequent masticating treatment, coating each particle of the fuel with a minute film of the binding solution 105 by subjecting the mixture to a masticating action until no accumulation of the binder as such exists in the mixture but the whole of said binder has been converted into a thin film extending throughout the mass of the 110 material, then forming the material into briquettes, completely removing the moisture therefrom and reducing the binder to 115 fibrous, fine-textured carbon.

4. A fuel briquette comprising a connected network of carbon supporting and containing within itself minute particles of 120 finely comminuted fuel and holding the same together in the form of a briquette, the briquette being waterproof and weatherproof and the result of a treatment whereby 125 finely comminuted particles of fuel mixed

with a water-soluble binding substance are subjected first to a masticating action until no accumulation of the binder as such exists in the mixture, but the whole of said binder

5 has been converted into a thin film extending throughout the mass of the material, said material having been then compressed

into briquette form and after briquetting, treated for the removal of moisture and carbonization of the binder.

10 In testimony whereof I have hereunto set my hand.

FELIX A. VOGEL.